

## UNITED STATES PATENT OFFICE.

LESTER KIRSCHBRAUN, OF CHICAGO, ILLINOIS.

## PROCESS FOR MAKING EMULSIFIED COMPOSITIONS.

No Drawing. Original application filed September 4, 1918, Serial No. 252,605. Divided and this application filed October 5, 1921. Serial No. 505,654.

*To all whom it may concern:*

Be it known that I, LESTER KIRSCHBRAUN, a citizen of the United States, residing in the city of Chicago, county of Cook, and 5 State of Illinois, have invented certain new and useful Improvements in Processes for Making Emulsified Compositions, of which the following is a specification.

This application is a division of an original 10 application, Serial No. 252,605, filed by me on September 4, 1918.

In an earlier application filed by me, to-wit: Serial No. 26,813, filed May 8th, 1915, I described a process of making an emulsified composition suitable for use with certain fibrous material. I have since discovered that in certain cases it may be advantageous to make a double emulsion. Heretofore in attempts to make waterproof 20 sheets, containing bitumen particularly as a continuous operation, on paper machines and the like, have experienced much difficulty in making a stock which would not stick to the machine. In the said prior 25 application I obviated this difficulty by making a non-sticky emulsified matrix composed of water and an emulsifying agent, such as clay of a colloidal character and a binder such as bitumen. In this matrix the 30 finely divided particles of the binder were in effect surrounded by a non-adhesive colloidal emulsifying agent, so that the material would pass readily over the paper machine without sticking. I have discovered 35 that in certain cases it may be desirable to form what in effect may be called a double emulsion. This double emulsion seems to permit of a more minute dispersion of the asphalt particles in the water 40 vehicle. Just exactly the action that takes place I am not at this time prepared to state. I have ascertained, however, that certain kinds of binders, as for example, some tars and oils, do not as readily emulsify with a clay paste as do others. Moreover, while a certain percentage of such 45 tars or oils might readily emulsify with the clay paste there seemed to be a limiting point at which no more tar or oil could be added and secure a satisfactory emulsion. I have discovered, however, that by making 50 a double emulsion I can overcome this objection.

The process of the present invention

may be described as follows: An adhesive 55 waterproof binder as bitumen, preferably in a hot liquid condition is placed in a suitable receptacle; to this liquid binder is gradually added a solution which may consist of water and soap; cheap resin soap 60 has been found satisfactory. This soapy solution is thoroughly mixed with the binder so as to produce an emulsion. In any event, this emulsified matrix is of a rather sticky character. Another way in 65 which this emulsion may be formed will be to dissolve a fatty acid such as oleic acid in a liquid binder and then add to this mixture a solution of suitable alkali such as common lye. This emulsion can be thinned 70 with water as desired. The mixture may vary in composition from two parts upwardly of soap to 100 parts of the binder. Care should be taken in adding the soap to 75 avoid an excess of alkali.

The first emulsion, which is a mobile liquid, is gradually added to an aqueous paste of water and material containing colloidal particles such as clay and the two 80 thoroughly mixed together to form a second emulsion. In forming this second emulsion, the weight of clay particles seem to coat the finely divided particles of the bitumen or other binder, and the result is an emulsified composition of a non-sticky 85 character.

I have above referred to making the first emulsion by the use of a fatty acid or saponifiable resin and later adding an alkali 90 solution. One advantage of making an emulsion in this way is that it permits the use of a very high melting point asphalt for a binder. For example, if an asphalt having say, 300 degrees F. melting point is desired to be used with the binder, it obviously cannot have an aqueous solution mixed with it when melted, for the reason that the melting point of the bitumen will be much above the boiling point of water. However, by first adding a fatty acid to 100 the high melting point binder, the latter is so softened or cut back by the fatty acid that it is a liquid at a temperature below the boiling point of water. The hot aqueous alkali solution can then be added and the alkali and fatty acid combined to form soap. This first emulsion can then be 105 mixed with a second emulsifying agent as

before stated. It will thus be seen that a very high melting point binder can be used. The utilization of a high melting point binder permits of the formation of a very hard and rubbery product.

After this double emulsion is formed, as above stated, it may, if desired, be combined with various kinds of fillers or fibrous materials and then moulded or sheeted as desired. As the water dries out of the mixture, the binder will coalesce, become adhesive and form a very tough and strong product.

While it may not be true in all cases, I have found that it is most desirable that in forming the first or primary emulsion that the aqueous solution containing the emulsifying agent be added to the binder rather than the binder to the aqueous solution, while in forming the second emulsion, the first emulsion is added to the second emulsifying agent rather than the reverse. With reference to the binders a wide variety of binders may be employed, either asphalts, natural or artificial coal tars, water gas tars, animal and vegetable pitches, hydrocarbon oils, drying oils, such as linseed oil, China-wood oil, wax tailings, wax paraffine, resin and the like. In some cases, the binder may consist of rubber dissolved in a suitable vehicle such as naphtha or benzol, which of course will ultimately evaporate. By the word "bituminous" as used in this specification and in the claims, is meant to include the various forms of binders referred to in the two preceding sentences.

I claim as my invention:

1. A process of making an emulsified matrix consisting in adding to a liquid waterproof adhesive binder a solution containing a substance which upon saponification becomes an emulsifying agent adding a saponifying substance thereto, and thoroughly mixing the solution and the binder to form an emulsion, then adding this emulsion to an aqueous paste containing colloidal particles and thoroughly mixing the paste and the primary emulsion to form a secondary composition.

2. A process of making an emulsified matrix consisting in adding to a liquid waterproof adhesive binder a saponifiable fluxing agent and then saponifying the liquid to produce an emulsion and adding the emulsion to a secondary colloidal emulsifying agent to produce a modified emulsion.

3. A process of the character described consisting in adding a fatty acid to a high melting point asphalt while the latter is in heated condition, thereby reducing the melting point, then adding a hot aqueous alkali solution, and then adding this mixture to an aqueous paste of colloidal clay.

4. A process of the character described, consisting in adding a saponifiable fluxing agent to a high melting point asphalt while the latter is in heated condition, thereby reducing the melting point saponifying said fluxing agent and then adding this mixture to an aqueous paste of colloidal clay.

LESTER KIRSCHBRAUN.